

## UNITED STATES PATENT OFFICE

2,408,971

## SLUSHING COMPOSITION

Gordon W. Duncan, Scotch Plains, N. J., assignor  
to Standard Oil Development Company, a cor-  
poration of Delaware

No Drawing. Application December 27, 1941,  
Serial No. 424,595

8 Claims. (Cl. 106—14)

1

The present invention relates to slushing compositions, particularly to those compositions applied to the surface of easily corrodible metals for arresting, preventing, and inhibiting the corrosion thereof.

The corrosion of the metal is considered to be the result of chemical reactions between the environment surrounding the metal, and the metallic surface due to differences in electro-motive forces in and about the surface of the metal. By coating metallic surfaces with an inert impervious film the development of these electro-chemical relations can be impeded and arrested and thus active corrosion prevented. The use of a slushing composition usually involves the formation of a viscous liquid or semi-solid layer on the metal which is easily removable from the surfaces over which it is spread by wiping with a cloth or flushing with a solvent.

In the application of slushing compositions the removal of adherent moisture offers some difficulty. In the fabrication of many metal machine parts it becomes necessary, as in the case of certain roller bearings, to electroplate a portion of the surface in an acid electroplating bath. After the electroplating operation is complete and the machine part removed from the bath, a washing operation is required to remove the adherent plating solution. It may then be necessary due to the character of the machine part to completely disassemble and dry it prior to the application of an anti-corrosion composition. Many other metal stock parts are water-washed during fabrication and this adherent moisture is customarily removed by oven drying over an ascertained period of time or by the application of a volatile liquid miscible with water and air-blowing. It would be much more convenient to apply a slushing compound capable of absorbing or dislodging adherent moisture directly from the metal. Articles that are manually moved or handled often are contaminated with moisture or perspiration from the hands of operating personnel. Subsequent slushing with a rust-proofing composition will not prevent rusting at these fingerprint marks unless the rust preventive is capable of absorbing or dislodging moisture directly from the metal.

It is an object of the present invention to provide an anti-corrosion composition or slushing compound for metals which will readily dislodge water and aqueous solutions from contact with metal surfaces. This and other objects will be apparent to those skilled in the art upon reading the following description.

It has now been found that the addition of a small amount, from 1 to 10%, of a compound partially or wholly soluble in both water and mineral oil distillates to an anti-corrosion composition or slushing compound results in an improved slushing compound having the characteristic of com-

pletely conditioning a ferrous metal surface against corrosion even in the presence of adherent water or aqueous solutions. Substances having the properties requisite for the purposes of the present invention and boiling within the range of from 100° C. to 300° C. possess the formula



where R is either hydrogen or an alkyl radical such as ethanol; alkylene represents a bivalent radical such as  $=CH_2$  (methylene),



etc., and R' is either hydrogen, an alkyl radical, such as methyl, ethyl, propyl, etc., or an aryl radical such as phenyl. In instances where both R and R' are hydrogen the alkylene radical should contain at least 4 and not more than 10 carbon atoms. Specific representative compounds of this class of materials are monomethyl ether of ethylene glycol, monobutyl ether of ethylene glycol, mono-ethyl ether of di-ethylene glycol, 1-phenoxy 2-hydroxy propane and 2-methyl 2,4-pentane diol.

The compositions of the invention are, therefore, improved slushing oil compositions which contain, in addition to a petroleum or fatty oil base and anti-rust agents, preferably of the metallic sulfonate type small amounts of both oil- and water-soluble dihydroxy alcohols (diols) of from 4 to 10 carbon atoms, mono-ethers of glycols or mono-ethers of ether-glycols. A specific instance of an anti-rust composition which is appreciably improved by the addition thereto of the compounds of this invention is that disclosed in Patent 2,182,992. The compositions therein disclosed are composed of a petroleum oil of lubricating oil consistency blended with a fatty compound, such as degras, and mahogany soap such as an alkaline metal soap of the oil-soluble sulfonates derived from petroleum by treating oils with concentrated sulfuric acid. The following formula is a specific example:

|                                                 | Per cent |
|-------------------------------------------------|----------|
| Petroleum oil (750 seconds Saybolt at 100° F.)  | 85       |
| 50% oil solution of sodium salts of oil-soluble |          |
| 50 sulfonic acids formed on treating petroleum  |          |
| stocks with concentrated sulfuric acid          | 10       |
| Degras                                          | 5        |

In compounding the compositions of the invention all that is necessary is to dissolve from 1 to 10%, preferably from 2 to 4%, of the additives previously described to a slushing oil composition such as disclosed in Patent 2,182,992 or other commonly employed slushing oil composition.

60 The efficacy of the slushing oil compositions of

this invention is evaluated by certain standard tests of which the water displacement test and corrosion test are the more important. In the water displacement test, sand blasted panels of hot rolled steel are dipped in tap water or other aqueous solution and are immediately immersed suspended in the slushing compounds for 100 seconds and the time required to displace the water or aqueous solution is noted by visual inspection. The panels are then suspended vertically for two hours in the atmosphere, then washed with naphtha, and examined for signs of corrosion. In a series of tests, the effects of several of the additive substances falling within the scope of the invention in solution in a slushing oil composition consisting of 80% petroleum solvent, 10% mahogany soap concentrate and 10% degras were investigated with the results given below. In all cases where corrosion does not occur within the two hour period the slushing compound film was found to give rust preventive results comparable to that obtained when a dry panel was coated with the slushing compound not containing the additive.

The compositions of this invention are effec-

petroleum fraction to which is added degras, a metal salt of oil-soluble sulfonic acids derived from petroleum by treating petroleum stocks with concentrated sulfuric acid and from 1 to 10% of a compound having the formula



wherein R is selected from the group consisting of hydrogen and alkyl radicals; and R' is selected from the group consisting of hydrogen, alkyl, and aryl radicals.

10 2. A composition according to claim 1 in which the compound is a mono-alkyl ether of a dihydric alcohol.

15 3. A composition according to claim 1 in which the compound is mono-butyl ether of ethylene glycol.

20 4. A composition according to claim 1 in which the compound is a dihydric alcohol of from 4 to 10 carbon atoms to the molecule.

5. A composition according to claim 1 in which the compound is 2-methyl 2,4-pentane diol.

6. A composition according to claim 1 in which the compound is an alkyl ether of an ether

25 glycol.

| Blend                                                                    | Aqueous displacement time, seconds | Corrosion with tap water at 2 hrs. | Corrosion with 0.1% HBr at 2 hrs. |
|--------------------------------------------------------------------------|------------------------------------|------------------------------------|-----------------------------------|
| Rust preventative composition                                            | No displacement 100 secs.          | Severe                             | Severe                            |
| Rust preventative composition                                            |                                    |                                    |                                   |
| Plus 4% methyl ether of ethylene glycol                                  | 50 secs.                           | None                               | None                              |
| Plus 4% butyl ether of ethylene glycol                                   | 12 secs.                           | do                                 | do                                |
| Plus 2% butyl ether of ethylene glycol                                   | 55 secs.                           | do                                 | do                                |
| Plus 4% ethyl ether of diethylene glycol                                 | 60 secs.                           | Trace                              | Slight                            |
| Plus 5% butyl ether of diethylene glycol                                 | 22 secs.                           | None                               | do                                |
| Plus 4% 1-phenoxy 2-hydroxy propane                                      | 45 secs.                           | do                                 | Trace                             |
| Plus 5% phenoxy propanol                                                 | 30 secs.                           | do                                 | Slight                            |
| Plus 5% phenoxy ethanol                                                  | 30 secs.                           | do                                 | do                                |
| Plus 4% 2-methyl 2,4-pentane diol                                        | 35 secs.                           | do                                 | None                              |
| Plus 4% secondary butyl alcohol                                          | 30 secs.                           | do                                 | do                                |
| 20% degras in Stoddard's solvent                                         | None                               | Severe                             | Severe                            |
| 20% degras in Stoddard's solvent plus 4% butyl ether of ethylene glycol. | Some displacement at 100 secs.     | Light                              | do                                |

tive for protecting finely polished surfaces and for all metal articles subject to corrosion resulting from adverse conditions of storage. Individual compositions have characteristics adapted for the particular uses for which they are to be employed. The consistency of the various compositions is determined by the surface requirements and the manner in which the compositions are to be applied to the surfaces to be protected. Thus, in the case of the protection of highly finished metal articles, such as cutlery and finely ground engine surfaces, the compositions may contain a volatile solvent in addition to the protective base. In other cases it is preferable to employ as anti-rust compositions, materials of consistencies similar to those of lubricating oils.

What is claimed is:

1. A slushing oil composition consisting of a

45 7. A composition according to claim 1 in which the compound is mono-butyl ether of di-ethylene glycol.

50 8. A slushing oil composition consisting of a viscous petroleum fraction to which is added 5% degras, 10% of a 50% oil solution of salts of oil-soluble sulfonic acids formed on treating petroleum stocks with concentrated sulfuric acid and from 2 to 4% of a compound having the formula



55 wherein R is selected from the group consisting of hydrogen and alkyl radicals; and R' is selected from the group consisting of hydrogen, alkyl, and aryl radicals.

60

GORDON W. DUNCAN.